

1

3,016,281

## PROCESS FOR TREATING CELLULOSIC TEXTILE MATERIAL WITH TRIACRYLYL-s-TRIAZINES

Edward L. Kropa, Greensboro, N.C., and Arthur S. Nyquist, Darien, Conn., assignors to American Cyanamid Company, New York, N.Y., a corporation of Maine

No Drawing. Filed Oct. 16, 1957, Ser. No. 690,454

10 Claims. (Cl. 8—116.2)

The present invention relates to a process for treating cellulosic textile materials to impart dimensional stability and wrinkle resistance thereto and to the textile materials so treated.

The impartation of dimensional stability and wrinkle resistance to textile fabrics heretofore has been accomplished by employing a wide variety of finishing agents and techniques. Most frequently, these properties are imparted to cellulosic textile fabric by applying thermosetting aminoplast resins, as for example, melamine-formaldehyde resins, urea-formaldehyde resins, including ethylene urea-formaldehyde resins, and their various alkylated derivatives, and curing the same in the presence of an acid curing catalyst. These di or multi-functional materials usually impart the properties of dimensional stability and wrinkle resistance to the textile material through the reaction between the labile hydrogens of the cellulosic hydroxyl group and the hydroxyl or alkoxy group of the aminoplast resin, with the splitting of water and/or alcohol. These reactions result in cross-linking of the cellulose fibers whereby the properties of wrinkle resistance and shrinkage control are accomplished.

For the most part, these finishing operations are highly satisfactory and do impart excellent wrinkle resistance and dimensional stability to the fabric so treated. They do, however, suffer certain shortcomings, principal among which is the deleterious effect imparted to fabric so finished by chlorine absorption, as when the fabric is washed in a media containing chlorine bleach. These effects manifest themselves as discoloration of the treated fabric or by adversely affecting the tensile strength of the treated fabric when it is scorched subsequent to chlorine bleaching.

Thermoplastic polymeric materials have been employed in the treatment of cellulosic textiles, as for example, binders for non-woven fabric, for the impartation of special "hand" effects, as for example, stiffness, either alone or in combination with other finishing materials, such as the aminoplast resins enumerated above. These thermoplastic textile finishes do not cross-link the cellulose fiber to impart dimensional stability and wrinkle resistance, in that their chemical structure restricts such activity. Any effect that finishes of this type impart to textile materials, such as wrinkle resistance and shrinkage control, appears to be the result of a purely physical association.

It is an object of the present invention to provide a process for the treatment of cellulosic textile materials to impart dimensional stability thereto and wrinkle resistance through the cross-linking of the cellulose fibers with a specific class of polyfunctional compound.

It is a further object of the present invention to provide cellulosic textile materials having improved dimensional stability and wrinkle resistance prepared in accordance with such a process.

These and other objects and advantages of the present invention will become apparent from the detailed description set forth hereinbelow.

According to the present invention, a process is provided for treating cellulosic textile materials to impart shrinkage control and wrinkle resistance thereto through cross-linking of the cellulosic fibers, which comprises

2

treating said textile material with a mixture comprising an aqueous solution of an alkaline compound as catalyst, and a triazine compound selected from the group consisting of those having the following general formula and the water-soluble bisulfite-modified adducts thereof:



wherein R<sup>1</sup>, R<sup>2</sup> and R<sup>3</sup> are members selected from the group consisting of hydrogen, methyl, ethyl, propyl and butyl. Also included in the treating mixture or blend is an inert solvent for the triazine compound, when the latter is not a water-soluble bisulfite-modified adduct. The alkaline compound employed as catalyst is present in an amount sufficient to catalyze the reaction between the cellulosic textile material and the treating compound. Thereafter, the fabric is dried and cured.

By "cellulosic textile material" as the term is used herein, it is meant fibers, films, filaments, formed fabrics, woven and non-woven, felted, or otherwise classified textile materials composed of at least 50% of cellulosic materials, which term is intended to include cotton, viscose rayon, jute, hemp, sisal, and the like, and mixtures thereof. For practical purposes, most applications are limited to formed textile materials or fabric, either woven or non-woven, composed of cotton or viscose rayon and thus for the most part the application of the present invention is directed to such fabrics.

The triazine compounds employable in the present invention may be termed 1,3,5-triacyl-s-triazines, and are disclosed, as is their method of manufacture and the preparation of their water-soluble bisulfite-modified adducts, in U.S. Patent No. 2,559,835, issued July 10, 1951, the disclosure of which is incorporated in the present specification by reference. They are preferably employed in their monomeric form, though certain low order polymers, including dimers, trimers and the like, may be employed. Of the compounds contemplated, those in which the R's are either hydrogen, methyl, ethyl or mixtures thereof are preferred and most efficiently employed.

The triazines coming within the general formula set forth hereinabove and which are contemplated by the present invention may be symmetrical or unsymmetrical. Thus, where R<sup>1</sup>, R<sup>2</sup> and R<sup>3</sup> are the same, the compound may be considered symmetrical and where they are different, the compounds may be considered unsymmetrical.

The following are illustrative of symmetrical compounds: 1,3,5-triacyl-s-triazine; 1,3,5-tris-(2-methylacryl)-hexahydro-s-triazine; 1,3,5-tris-(2-ethylacryl)-hexahydro-s-triazine; 1,3,5-tris-(2-propylacryl)-hexahydro-s-triazine; 1,3,5-tris-(2-isopropylacryl)-hexahydro-s-triazine; 1,3,5-tris-(2-butylacryl)-hexahydro-s-triazine; and 1,3,5-tris-(2-isobutylacryl)-hexahydro-s-triazine. As illustrative of the unsymmetrical triazines, 1-acryl-3,5-bis-(2-ethylacryl)-hexahydro-s-triazine and 1-(2-butylacryl)-3,5-bis-(2-ethylacryl)-hexahydro-s-triazine may be employed. These compounds are applied to the cellulose textile in amounts from between 3 and 25% and preferably from between 5 and 15%, based on the dry weight of the textile fabric. These triazines may be employed singly or in combination with one another in accordance with the present invention.

The aqueous solution of alkaline compounds employed as catalysts in the present process may be sodium hydroxide, potassium hydroxide or lithium hydroxide, sodium carbonate, sodium bicarbonate, choline, morpholine, triethanolamine, or any combination thereof. It is essential to the present process that a moderate to strong alkali catalyst material be employed, in order to effect the desired results, and that it be present in an amount sufficient to catalyze the reaction between the cellulose and the triazine. It has been determined that the treating composition should have a pH above 8 and preferably above 9, depending upon the nature of the alkaline catalyst compound employed.

When the water-insoluble triazines are employed, a solvent must be used therewith. Such a solvent must function both as a solvent for said triazine and must further be inert with respect thereto and the treating medium. As suitable classes of solvents, broadly ethers and ketones may be mentioned. Specifically, methyl ethyl ketone and acetone may be cited by way of example, and dioxane is the preferred solvent in the present process. Other solvents which may be employed are dimethyl formamide, ethylene carbonate, and the like. These solvents and their equivalents may be employed singly or in combination with one another.

With certain of the solvents, as for example, acetone, the triazines of the present invention are not fully soluble therein. The use of strong alkaline compounds such as sodium hydroxide in such treating compositions, in addition to functioning as a catalyst for the reaction between the cellulose and triazines, functions as a solubilizing agent, rendering the triazine fully soluble in the acetone.

In accordance with the present invention, the triazine is preferably dissolved in the solvent, as for example, dioxane, and the alkaline compound employed as catalyst, as for example, sodium hydroxide, is dissolved in water. The respective solutions are then blended and the textile material treated therewith.

As has been previously pointed out, the treating composition or mixture should have an alkaline pH above 8, but preferably is above 9. It may generally be said that the pH value of the treating mixture is not significant, except insofar as it is a measure of the necessary amount of alkaline compound present as catalyst for the reaction between the cellulose and the triazine. Thus, where the amount of catalyst present is sufficient to provide a treating composition with a pH above 8, and preferably above 9, the presence of sufficient catalyst is indicated. Expressed as percent of the total treating composition, the alkaline compound present as catalyst should be present in an amount of less than 5% of the total weight of treating composition and preferably from between about 0.05-4% thereof. Based on the weight of the triazine, an amount of from between 5 and 15% should normally be employed. If the amount of catalyst is insufficient to produce such pH values, the reaction proceeds too slowly and undesirable side reactions have been known to occur. If too much alkali is present, undesirable effects such as discoloration of the treating textile material upon drying and curing are incurred.

The composition of the present invention may be applied by any of the conventional textile finishing techniques, as for example, padding, spraying, immersion, and the like. The process of the present invention preferably employs padding techniques.

The mixture of the present invention is applied as by padding to the cellulose textile material so as to impart from between about 3 and about 25% and preferably from between about 5 and 15% of the triazine to the textile fabric, based on the dry weight of the fabric. Thereafter, the fabric is dried and cured. For the most part, the times and temperatures of drying and curing are readily determinable. Generally speaking, the time of drying and curing is inversely proportioned to the temperatures employed. Thus, by way of example, drying and curing

may be accomplished by drying the treated fabric, as for example, at 200° F. until dry to the touch, followed by curing for from 3 minutes at 290° F. to 0.5 minute at 450° F. If it is preferred to dry and cure in a single operation, times and temperatures of from 8 minutes at 250° F. to 1 minute at 450° F. may be employed.

In order that the present invention may be more fully understood, the following examples are given primarily by way of illustration. No details found therein should be construed as limitations on the present invention, except as they appear in the appended claims. All parts and percentages are by weight unless otherwise indicated.

#### EXAMPLE 1

15 Fifteen parts of 1,3,5-triacrylyl-hexahydro-s-triazine are dissolved in 150 parts of dioxane. Blended with this solution is an aqueous solution of 1.5 parts of 100% sodium hydroxide in 90 parts of water. The pH of the blend was above 9.

20 80" x 80" cotton percale was padded through the solution so as to apply a 100% wet pick-up. Thereafter, the treated fabric was dried and cured in a single operation for 6 minutes at 290° F. The amount of triazine applied to the cloth was about 6%, based on the dry weight of the fabric.

25 The results of this application will be reported in Table I set forth hereinbelow.

#### EXAMPLE 2

30 Twenty-five parts of 1,3,5-tris-(2-methylacrylyl)-hexahydro-s-triazine were dissolved in 150 parts of acetone. Blended with this solution was 2 parts of 100% potassium hydroxide in 90 parts of water. In this mixture, the potassium hydroxide functioned as a solubilizing agent for the triazine in the acetone medium. The pH of the blended composition was above 9.

35 80" x 80" cotton percale was padded through the treating composition to a 100% wet pick-up. Thereafter, the treated fabric was dried and cured in a single operation for 6 minutes at 290° F.

40 This treatment resulted in a pick-up of about 9%, based on the dry weight of the cotton fabric.

45 The results of this application are reported in Table I hereinbelow.

Table I

| Application                     | Shrinkage (1 wash), percent | Dried Wrinkle Recovery (both warp and fill), degrees |
|---------------------------------|-----------------------------|------------------------------------------------------|
| Example 1.....                  | 1.1                         | 223                                                  |
| Example 2.....                  | 1.0                         | 235                                                  |
| Control (untreated fabric)..... | 5.6                         | 145                                                  |

55 The above results clearly indicate that the application of the triazines according to the process of the present invention results in the improvement of the dimensional stability and in the wrinkle recovery of the treated fabric. In addition, in both Examples 1 and 2, the treated fabrics had a soft "hand" and were not stiff, indicating that the triazine did not polymerize on the surface, but cross-linked within the cellulose fibers. Further, the treated fabric did not discolor as a result of chlorine absorption.

60 In the above table and subsequently in the present specification, the wash for the treated cotton fabric and control fabric involves washing the fabric for one hour in 0.1% soap and 0.1% soda ash at 160° F. in an agitator washer, followed by a thorough rinsing in water at 160° F. Shrinkage control, the measure of dimensional stability imparted, was determined by measuring the treated samples before and after washing and drying and expressing the change in dimensions as a percentage of the original dimensions.

65 Wrinkle recovery was determined by the use of a

Monsanto crease-angle recovery tester, and the values reported are in degrees. The washes and tests are standard in the textile finishing industry, and are further amplified in the 1956 Yearbook of "The American Association of Textile Chemists and Colorists," on page 138. 5

## EXAMPLE 3

To a solution consisting of 10 parts of 1,3,5-triacrylyl-hexahydro-s-triazine in 100 parts of dioxane a solution of 1 part of 100% sodium hydroxide in 60 parts of water is added followed by blending. The composition has a pH above 9. 10

This composition is applied to rayon challis by immersion of the challis in the treating composition for from 2 to 3 minutes. The treated fabric is then padded and pinned to size. The wet pick-up of the treating solution is about 100%. The treated-challis is air dried for about 1½ hours and then dried and cured for 6 minutes at 290° F.

Thereafter, the treated challis and an untreated control were washed in 0.1% soap at 100° F. in an agitator washer, followed by thorough rinsing in water at 100° F. and each of the samples were measured for shrinkage control in accordance with the procedure outlined hereinabove.

The treated fabric underwent shrinkage of 8% and the untreated sample had a shrinkage of about 19%, thus indicating that the treatment of rayon challis according to the present invention results in a positive and substantial improvement in shrinkage control.

In U.S. Patent No. 2,559,694 (which patent is incorporated by reference herein) it is disclosed that compounds of the type generally contemplated for use in the present invention have heretofore been used in conjunction with textile materials. Thus, for example, it is broadly disclosed that 1,3,5-triacrylyl-hexahydro-s-triazine may be polymerized in the presence of textile materials. In this contemplated reaction, the triazine is polymerized in the presence of the textile material through the initiating action of a catalyst for the polymerization, as for example, of benzoyl peroxide or hydrogen peroxide. Such a treatment does not impart dimensional stability and wrinkle resistance through a cross-linking of the fibers of the textile material, but alternatively results in a physically associated non-durable polymer finish which renders the fabric stiff.

In order to illustrate the significance of the difference in the process of the present invention over the disclosure of U.S. Patent No. 2,559,694, the sodium bisulfite adduct of 1,3,5-triacrylyl-hexahydro-s-triazine was prepared in accordance with the procedure defined in Example 4 of said patent. Three applications were then made to 80" x 80" cotton percale as follows:

(a) 5% solids of the bisulfite adduct was boiled with hydrogen peroxide in water for 10 minutes and then applied to the cotton percale, followed by drying and curing in accordance with the procedure set forth in Example 6 of the said patent.

(b) The same procedure as in (a) above was followed except that the step of boiling the bisulfite adduct preliminary to application to the percale was omitted.

(c) 10% solids of the bisulfite adduct containing 10% NaOH based on the adduct solids was applied to the percale, and the cloth was dried 2 minutes at 225° F. and cured 1.5 minutes at 350° F.

The treated fabric and untreated control were then tested for wrinkle recovery, hand and stiffness. The results are recorded in Table II hereinbelow. The wrinkle recovery values are in degrees, as determined by a Monsanto crease-angle tester. The "hand" values are relative and determined by a skilled operator actually feeling the fabric. The stiffness values reported are obtained by employing a Gurley stiffness tester, and the values reported are in milligrams and represent total warp plus filling. The higher the value, the stiffer the fabric.

6  
Table II

| Application       | Hand     | Gurley Stiffness | Wrinkle Recovery (Total W + F) |
|-------------------|----------|------------------|--------------------------------|
| (a) (initial)     | Stiff    | 42               | 144                            |
| (a) (1-hour wash) | Soft     | 23               | 150                            |
| (b)               | Soft     |                  | 144                            |
| (c)               | SL. firm |                  | 206                            |
| Untreated         | Soft     | 14               | 150                            |

From this data the following conclusions may be arrived at:

(1) Polymerization of the bisulfite adduct of 1,3,5-triacrylyl-hexahydro-s-triazine prior to application to the cotton percale effects a non-durable increase in fabric stiffness. From this it may be concluded that the resin is on the fabric as a coating and probably not chemically bound thereto.

(2) The in situ polymerization of the bisulfite adduct does not occur unless the pre-polymerization step is carried out. This is evidenced by the fact that no hand modification of the fabric treated as in (b) was encountered. Thus, if the adduct polymerized to form a coating it would have rendered the fabric stiff. It should also be noted that the procedure of (b) apparently did not react or cross-link with the fabric in that no improvement in wrinkle recovery was recorded.

(3) Application of the unpolymerized bisulfite adduct with a catalyst employable in the process of the present invention improves substantially the wrinkle recovery of the treated fabric, and does not significantly stiffen the hand of the fabric. This may be interpreted to mean that in accordance with the process of the present invention the cellulose fibers are cross-linked.

In a particular disclosed application according to the above-cited reference, 1,3,5-triacrylyl-hexahydro-s-triazine is rendered water soluble by modification with a sulfite group and is then polymerized in the presence of percale through the initiating activity of a hydrogen peroxide catalyst. The treated fabric is stiff, which may properly be interpreted as a strong indication of the surface polymerization of the triazine on the percale, as opposed to the entering of the fibers and cross-linking of the same through the saturation of the double bonds of the triazine.

Since the triazines of the present invention are employed as monomers or lower order polymers, and since the finished fabric has dimensional stability, wrinkle resistance and a soft hand, it is believed that a major portion of the triazine enters into the cellulose fiber to cross-link the same. It is believed that the reaction may be represented as follows:



As has been pointed out hereinabove, the present process is directed primarily to the improvement of dimensional stability and wrinkle resistance of cellulosic fabrics.

While the present process effects reaction with cellulosic textile materials of the type contemplated and described hereinabove, these materials may, of course, be mixed with other non-cellulosic materials. Thus, for example, the cellulosic textile material may be blended with nylon, polyester fibers, acrylic fibers, and other synthetic materials. Normally, unless the treated fabric contains at least 50% and preferably more of cellulosic textile material, the effect of the process is significantly reduced.

Where compatible, the treating composition of the present invention may be employed with pigments, dyes, lubricants, wetting agents and the like, and to some extent other finishing resinous materials, as for example, aminotriazine-formaldehyde resins such as melamine-formaldehyde resins, ethylene urea-formaldehyde resins, urea-formaldehyde resins and the alkylated derivatives thereof.

We claim:

1. A process for treating cellulosic textile material to impart shrinkage control and wrinkle resistance thereto through cross-linking of the cellulosic fibers, which consists essentially in treating said textile material in its entirety with a composition comprising an aqueous solution of an alkaline compound as a catalyst and a triazine compound selected from the group consisting of those having the following general formula:



wherein  $\text{R}^1$ ,  $\text{R}^2$  and  $\text{R}^3$  are selected from the group consisting of hydrogen, methyl, ethyl, propyl, butyl and the water-soluble bisulfite-modified adducts thereof, said alkaline catalyst being present in an amount sufficient to catalyze a reaction between the cellulose and said compound, and thereafter drying and curing the treated fabric.

2. A process for treating cellulosic textile material to impart shrinkage control and wrinkle resistance thereto through cross-linking of the cellulosic fibers, which consists essentially in treating said textile material in its entirety with a composition comprising an aqueous solution of an alkaline compound as catalyst and a solvent solution of a triazine having the following general formula:



wherein  $\text{R}^1$ ,  $\text{R}^2$  and  $\text{R}^3$  are selected from the group consisting of hydrogen, methyl, ethyl, propyl and butyl, said solvent being inert with respect to said triazine, said alkaline catalyst being present in an amount sufficient to catalyze a reaction between the cellulosic material and said compound said compound being applied so as to impart from between 3 and 25% by weight thereof to the material, based on the weight of the material, and thereafter drying and curing the treated fabric.

3. A process according to claim 2 in which the alkaline catalyst is sodium hydroxide,  $\text{R}^1\text{-R}^3$  are hydrogen, and the solvent for the triazine is dioxane.

4. A process according to claim 2 in which  $\text{R}^1\text{-R}^3$  are methyl.

5. A process according to claim 2 in which  $\text{R}^1\text{-R}^3$  are ethyl.

6. A process according to claim 2 in which the cellulosic material is cotton.

7. A process according to claim 2 in which from between 5 and 15% of the triazine is applied to the material based on its dry weight.

8. A process for treating cellulosic textile material to impart shrinkage control and wrinkle resistance thereto

through cross-linking of the cellulosic fibers, which consists essentially in treating said textile material in its entirety with a composition comprising an aqueous solution of an alkali metal hydroxide catalyst and a water-soluble bisulfite adduct of a triazine having the following general formula:



wherein  $\text{R}^1$ ,  $\text{R}^2$  and  $\text{R}^3$  are selected from the group consisting of hydrogen, methyl, ethyl, propyl and butyl, said alkali metal hydroxide catalyst being present in an amount sufficient to catalyze a reaction between the cellulosic material and said compound said compound being applied so as to impart from between 3 to 25% by weight thereof to the material, based on the weight of the material, and thereafter drying and curing the treated fabric.

25 9. Cellulosic textile material having improved shrinkage control and wrinkle resistance through cross-linking of the cellulosic fibers with a compound selected from the group consisting of those having the following general formula:



30 40 and the bisulfite-modified adducts thereof, in which  $\text{R}^1$ ,  $\text{R}^2$  and  $\text{R}^3$  are selected from the group consisting of hydrogen, methyl, ethyl, propyl and butyl.

10. Cellulosic textile material having improved shrinkage control and wrinkle resistance through cross-linking 45 of the cellulosic fibers with from between 3 and 25% of a compound selected from the group consisting of those having the following general formula:



50 55 and the bisulfite-modified adducts thereof, in which  $\text{R}^1$ ,  $\text{R}^2$  and  $\text{R}^3$  are selected from the group consisting of hydrogen, methyl, ethyl, propyl and butyl.

#### References Cited in the file of this patent

#### UNITED STATES PATENTS

|    |           |                      |                |
|----|-----------|----------------------|----------------|
| 65 | 1,886,480 | Haller et al. _____  | Nov. 8, 1932   |
|    | 2,301,509 | Bock et al. _____    | Nov. 10, 1942  |
|    | 2,332,047 | Bock et al. _____    | Oct. 19, 1943  |
|    | 2,559,694 | Zerner et al. _____  | July 10, 1951  |
|    | 2,559,835 | Zerner et al. _____  | July 10, 1951  |
|    | 2,568,620 | Gresham et al. _____ | Sept. 18, 1951 |
|    | 2,643,958 | Kleiner et al. _____ | June 30, 1953  |
| 70 | 2,651,631 | Zerner et al. _____  | Sept. 8, 1953  |

UNITED STATES PATENT OFFICE  
CERTIFICATION OF CORRECTION

January 9, 1962

Patent No. 3,016,281

Edward L. Kropa et al.

It is hereby certified that error appears in the above numbered patent requiring correction and that the said Letters Patent should read as corrected below.

corrected below.  
Column 6, lines 59 to 63, the formula should appear as  
shown below instead of as in the patent:



column 8, line 22, for "to", second occurrence, read -- and --.

Signed and sealed this 12th day of June 1962.

(SEAL)

Attest:

## ERNEST W. SWIDER

**Attesting Officer**

DAVID L. LADD

Commissioner of Patents